

BEST AVAILABLE COP'

# UNITED STATES PATENT OFFICE.

SHERARD OSBORN COWPER-COLES, OF LONDON, ENGLAND, ASSIGNOR OF  
ONE-HALF TO THE REFLECTOR SYNDICATE, LIMITED, OF SAME PLACE.

## MANUFACTURE OF REFLECTORS.

SPECIFICATION forming part of Letters Patent No. 660,416, dated October 23, 1900.

Application filed November 7, 1898. Serial No. 695,782. (No specimens.)

*To all whom it may concern:*

Be it known that I, SHERARD OSBORN COWPER-COLES, engineer, a subject of the Queen of Great Britain, residing at Grosvenor Mansions, Victoria street, London, England, have invented new and useful Improvements in the Manufacture of Reflectors, of which the following is a specification.

This invention relates to improvements in  
10 the manufacture of parabolic reflectors by  
the electrodeposition of the same on suitable  
molds.

An important feature of the present invention consists in the employment of molds of  
15 speculum metal instead of the glass molds heretofore used, thus enabling a highly-polished, truly-shaped, and electrically-conductive surface to be obtained without the special treatment necessary where glass is used.  
20 A further important feature of the invention consists in the application of a reflecting and protecting surface of platinum to the electrically-deposited reflector.

According to the said invention the specu-  
25 lum metal is cast in an iron mold heated al-  
most to the melting-point of the said metal, which may advantageously consist of tin, fifteen parts, copper, thirty-two parts, and arsenic, one part; or tin, one part, and copper,  
30 two parts. This metal is poured carefully into the mold through a central feed-opening or runner, so as to insure a sound casting free from blowholes, the edge of the mold being left open. The casting is then removed from  
35 the mold and is brought in any convenient manner to the true geometrical shape required for the finished mold, after which it is pro-  
vided with as high a polish as possible. It is  
then coated with a thin film of beeswax dis-  
40 solved in a suitable solvent to facilitate the  
removal of the mirror from the mold. This  
film of wax is so thin that it does not act as an  
insulator to the mold and does not therefore  
require metallizing. The body of the reflec-  
45 tor is then electrically deposited on the mold  
in one or more layers, the surface next the  
mold acquiring a highly-polished and true  
surface corresponding to that of the mold.  
When the deposition has been carried on to  
50 the required extent, it is stopped and the re-  
flector-backing and mold detached from one

another, which may be readily done by heating them slightly, (preferably by dipping them in hot water,) when the difference in expansibility will cause them to separate. 55 That surface of the reflector which was adjacent to the mold is then cleaned chemically—for example, with a solution of potassium cyanid or hydrate—and the reflecting and protecting surface of platinum, palladium, or chromium is applied to it by means of electrical deposition.

The bath used for the electrodeposition of the platinum may be composed of freshly-precipitated double chlorid of platinum and 65 ammonium dissolved in a boiling concentrated solution of neutral citrate of sodium. The solution is preferably used in the cold state and should contain about one and one-half ounces of metal to the gallon. The current 70 should have a density of about three amperes per square foot of cathode-surface, and the difference of potential between the terminals of the depositing-cell should be about 0.75 of a volt. 75

What I claim is—

1. A process for manufacturing a reflector by electrodeposition, consisting in coating the surface of a metal mold with a film of wax which is so thin that it does not act as 80 an insulator, electrolytically depositing the metal body of the reflector on said coated surface, separating the mold and body by varying the temperature, chemically cleaning the surface of the body that was in contact with the mold, and then electrolytically depositing a reflecting and protecting surface on said cleansed surface, substantially as described. 85

2. A process for manufacturing a reflector 90 by electrodeposition, consisting in coating the surface of a speculum-metal mold with a film of wax which is so thin that it does not act as an insulator, electrolytically depositing the metal body of the reflector on said coated surface, separating the mold and body by immersing them in hot water, chemically cleaning the surface of the body that was in contact with the mold, and then electrolytically depositing a reflecting and protecting surface on said cleansed surface, substantially as described. 95 100

process for manufacturing a reflector by electrodeposition, consisting in coating the surface of a speculum-metal mold with a film of wax which is so thin that it does not act as an insulator, electrolytically depositing the metal body of the reflector on said coated surface, separating the mold and body by immersing them in hot water, chemically cleansing the surface of the body that was in contact with the mold, and then electrolytically depositing a reflecting and protecting surface of platinum from a solution of freshly-precipitated double chlorid of platinum and ammonium in a concentrated solution of neutral citrate of sodium on said cleansed surface, substantially as described.

4. A process for manufacturing a reflector by electrodeposition, consisting in coating the surface of a speculum-metal mold with a film of wax which is so thin that it does not act as an insulator, electrolytically deposit-

ing the metal body of the reflector on said coated surface, separating the mold and body by immersing them in hot water, chemically cleansing the surface of the body that was in contact with the mold, and then electrolytically depositing a reflecting and protecting surface of platinum from a solution of freshly-precipitated double chlorid of platinum and ammonium in a concentrated solution of neutral citrate of sodium on said cleansed surface, substantially as described.

In testimony whereof I have hereunto set my hand, in presence of two subscribing witnesses, this 7th day of October, 1898.

SHERARD OSBORN COWPER-COLES.

Witnesses:

GEO. P. S. KELSEY,  
WALTER E. ROCHE.